

Nov. 7, 1939.

R. E. BURK ET AL

2,179,208

MANUFACTURE OF IMPROVED ASPHALTS

Filed Nov. 23, 1936



INVENTOR.

Robert E. Burke and  
BY Charles H. Whitacre  
Day, Oberling & Day  
ATTORNEYS

## UNITED STATES PATENT OFFICE

2,179,208

## MANUFACTURE OF IMPROVED ASPHALTS

Robert E. Burk and Charles H. Whitacre, Cleveland, Ohio, assignors to Standard Oil Company, Cleveland, Ohio, a corporation of Ohio

Application November 23, 1936, Serial No. 112,348

5 Claims. (Cl. 196—74)

In manufacturing asphalt, it has been the custom to blow the petroleum residuum with air, and maintain the temperature at about 300—500° F. The procedure is very tedious, requiring a long duration of action in order to bring the material to useable characteristics of high melting point and low penetration. Although enormous quantities of oxygen are brought into relation with the hydrocarbon material, there is not a great increase in the oxygen content, and the action is largely a dehydrogenation and conjoining of hydrocarbon molecules. We have now found that particularly effective action in thickening up the material to desirable penetration and melting point can be obtained without the cumbersome and time-consuming air-blowing, and the entire operation can be completed in a fraction of the time heretofore necessary, the products being also superior.

To the accomplishment of the foregoing and related ends, the invention, then comprises the features hereinafter fully described, and particularly pointed out in the claims, the following description and the annexed drawing setting forth in detail certain illustrative embodiments of the invention, these being indicative however, of but a few of the various ways in which the principle of the invention may be employed.

In said annexed drawing the sole figure is a diagrammatic showing on the order of a process flow sheet.

The stock to be worked up, a heavy petroleum oil residue, which we designate the residuum, is in accordance with the invention heated with air and a small or catalytic amount of a polymerizing catalyst. The temperature of treatment may be 225—450° F. Desirably, the material is suitably stirred or agitated. The time of treatment is short, as for instance 20 to 300 minutes, e. g., 90 minutes with 5 per cent  $FeCl_3$  at 260—280° F. As catalysts, we may employ a small amount of acid, as for instance chloro-sulphonic, phosphoric, fluoboric, hydrochloric, nitric or sulphuric acids, and halides, as ferric chloride, aluminum bromide, chloride, iodide, halides similarly of copper, tin, zinc, antimony, arsenic, titanium, etc., hydroxides of sodium, potassium, etc., calcium oxide, sodium carbonate, metallic sodium, nitrogen bases, ozonides in minute amounts and peroxides in minute amounts. Particularly desirable catalysts are the acid acting catalysts, as sulphuric acid, ferric chloride, halides of aluminum, copper, tin, zinc, antimony, arsenic, titanium, boron fluoride, chlorsulphonic,

phosphoric, fluoboric, hydrochloric, nitric acids, etc.

In some instances, it is desirable to subject the petroleum residuum first to an air-blowing, maintaining the temperature at about 450° F. for about 600 minutes, the material being agitated by the injected air or other suitable means, and then the air-blowing is discontinued and the polymerizing catalyst is incorporated, e. g., 0.5 per cent  $AlCl_3$  at a temperature of about 250° F. and the heating is maintained at 300—400° F. for 20 to 30 minutes. Such air-blowing stage can be operated to some desired penetration standard, as for instance 92 penetration at 77° F., and then the polymerization treatment is applied.

As an example: A petroleum residuum having initially a penetration of 200 at 77° F., is heated with 1.5 per cent of ferric chloride at a temperature of 350° F., for 60 minutes. The product has a penetration of 115 at 77° F. and ductility 16 at 39° F. and 72.5 at 77° F.

As another example: Similar petroleum residuum is air-blown at a temperature of about 450° F. for about 12 hours, and this material is then heated with 0.5 per cent of sulphuric acid at 350° F. for 30 minutes. The product has a melting point of 137.5, ductility at 39° F. 3.5, ductility at 77° F. 29, penetration at 32° F. 17, penetration at 77° F. 44, penetration at 115° F. 155, and susceptibility coefficient 3.1 (the susceptibility coefficient indicates the ratio of penetration at different temperatures, viz., S equals the penetration at 115 minus the penetration at 32 over the penetration at 77).

As another example: A petroleum residuum is similarly air-blown first, and then is heated with 0.9 percent of boron fluoride in a  $BF_3$ —ether mixture at a temperature of 400° F. for 15 minutes. The product has a melting point of 140° F., ductility at 38° F. 4, and at 77° F. 21, penetration at 32° F. 19, and at 77° F. 47, and at 115° F. 146, and a susceptibility coefficient of 2.7.

As another example: The petroleum residuum is similarly first air-blown as above, and then is heated with 0.5 per cent of  $FeCl_3$  at 400° F. for 30 minutes. The product has a melting point of 130° F., ductility at 39° F. 4, and at 77° F. 30, penetration at 32° F. 17, and at 77° F. 51, and at 115° F. 192, and susceptibility factor 3.4.

Asphalts produced according to the present invention have particularly shiny black surfaces, and are not buttery or short in consistency as has been the characteristic of asphalts from blended stocks. They also have higher melting

points at a given penetration, at say 77° F., than a customary asphalt, and better susceptibility coefficients.

Other modes of applying the principle of the invention may be employed, change being made as regards the details described, provided the features stated in any of the following claims, or the equivalent of such, be employed.

We therefore particularly point out and distinctly claim as our invention:

- 10 1. A process of making asphalt, which comprises air-blowing a petroleum residuum in the absence of an added catalyst while maintaining the temperature at 300-500° F., for one to thirty or more hours, then heating the material at a temperature at least 300° F. with a small amount of a polymerizing catalyst.
- 15 2. A process of making asphalt, which comprises air-blowing a petroleum residuum in the absence of an added catalyst while maintaining the temperature at 300-500° F., for one to thirty or more hours, then heating the material at a temperature at least 300° F. with a small amount of an acid-acting catalyst.

3. A process of making asphalt, which comprises air-blowing a petroleum residuum in the absence of an added catalyst while maintaining the temperature at 300-500° F., for one to thirty or more hours, then heating the material at a 5 temperature at least 300° F. with a catalytic amount of sulphuric acid.

4. A process of making asphalt, which comprises air-blowing a petroleum residuum in the absence of an added catalyst while maintaining 10 the temperature at 300-500° F., for one to thirty or more hours, then heating the material with a catalytic amount of boron fluoride.

5. A process of making asphalt, which comprises air-blowing a petroleum residuum in the absence of an added catalyst while maintaining 15 the temperature at 300-500° F., for one to thirty or more hours, then heating the material with a catalytic amount of ferric chloride. 20

ROBERT E. BURK.  
CHARLES H. WHITACRE.